

July 15, 1952

P. S. BLICKENSDERFER

2,603,593

ELECTRODEPOSITION OF METALS

Filed Jan. 8, 1946

4 Sheets-Sheet 1



Philip S. Blickensderfer

Frederick G. L. Boyer

Attorneys

July 15, 1952

P. S. BLICKENSDERFER

2,603,593

Filed Jan. 8, 1946

## ELECTRODEPOSITION OF METALS

4 Sheets-Sheet 2



Philip S. Blickensderfer Inventor

Frederick G. L. Bayer Attorney

July 15, 1952

P. S. BLICKENSDERFER

2,603,593

ELECTRODEPOSITION OF METALS

Filed Jan. 8, 1946

4 Sheets-Sheet 3



July 15, 1952

P. S. BLICKENSDERFER

2,603,593

ELECTRODEPOSITION OF METALS

Filed Jan. 8, 1946

4 Sheets-Sheet 4



INVENTOR  
Philip S. Blickensderfer  
BY  
Frederick G. L. Boyer  
ATTORNEY

## UNITED STATES PATENT OFFICE

2,603,593

## ELECTRODEPOSITION OF METALS

Philip S. Blickensderfer, Hamilton, Ohio, assignor  
to The Champion Paper and Fibre Company,  
Hamilton, Ohio, a corporation of Ohio

Application January 8, 1946, Serial No. 639,873

21 Claims. (Cl. 204—16)

1

This invention relates to the electrolytic deposition of metals and has particular value in the local deposition of metals for the filling of holes, pits, worn or peeled areas, cracks and scratches, the uniting of separate pieces, or for other purposes, and it has particular utility in securing and maintaining superior continuity and uniformity and a high degree of perfection in extensive smooth highly polished solid or plated metal surfaces.

Articles such as tools, gages, etc., in which a steel article has been provided with a wearing surface of chromium, frequently become worn or damaged in service so that the chromium surfacing must be built up or replaced. If the plate has been worn or has peeled off down to the base metal in even a small part of the plated area, or if it becomes so in the preparation, whether mechanical or electrolytic, for replating, it has heretofore been considered necessary to strip off all of the chromium and start afresh. Solid or plated metallic surfaces of rotating drums, endless metal belts, etc. for use in the casting of cellulosic or other films, of coating on paper (as described in Patent No. 1,719,166) or the like, require a high degree of perfection in uniformity, smoothness, continuity, and freedom from cracks, scratches, holes, pits, or other defects, so that considerable difficulty has heretofore been experienced in securing the required degree of perfection throughout the area of surfaces as large as are required for commercial casting operations. Rolled and cast metals of the necessary surface area are all subject to the presence of voids, slag inclusions, and the like, which even when extremely small are, unless cleaned out, filled to the edges, and polished over, sufficient to impair if not to completely destroy the value of the surface for casting purposes. Electroplating, particularly with chromium which otherwise is a highly desirable material for a casting surface, ordinarily does not cover, but rather accentuates such defects in the base metal, and also frequently exhibits other defects not previously apparent. The customary method of stripping off all of the chromium and replating whenever the base metal becomes exposed is consequently not satisfactory for the preparation of such extensive surfaces with the required degree of freedom from even minute defects, since the replating cannot be depended upon to reduce the total number of such defects. Even when a satisfactory surface has once been secured the problem still remains, since in continued use such surfaces are always subject to damage such as scratches, dents, nicks, etc., one of which is frequently suf-

2

ficient to completely destroy the utility of a casting surface a great many square feet in area. Endless flexible belts, even if made of electro-formed strip are still subject to objectionable pin-holes, etc. and are additionally subject in service to such damages as dents, tears, and the like, as well as requiring splicing to give them their endless form.

The primary object of the present invention is to provide a method by which holes, pits, cavities, dents, cracks, tears, and the like in metallic surfaces can be electrolytically filled, so that after the patches are cut down to the surface level, the degree of perfection of the surface is substantially the same as though the defect had never existed. An allied object is to provide such a method for patching worn or defective electroplate, particularly of chromium. A further object is to provide a method for electrodepositing an adherent layer of chromium onto a surface composed partly of iron and partly of chromium whereby to make possible the patching as stated of holes, pits, cavities, etc. in a chromium plated surface in cases where these defects extend through the layer of chromium into the ferrous base metal. Another object is to provide a method whereby discrete parts may be joined as for the purpose of patching large holes (which may be due to cutting out damaged or defective portions) in the metal belts or sheets by insertion of a coplanar inlay of similar metallic sheet in the hole and electrolytically uniting this with the surrounding metal to form a single substantially homogeneous sheet. Other objects and advantages of the invention will be made apparent by the following description:

I have now found it possible, in accordance with the present invention as hereinafter more fully described, to successfully accomplish the aforesaid objects and fill even minute holes, pits, scratches, cracks, etc. in a finished solid or plated metallic surface, so that a surface unfit for use because of such defects can be rendered smooth, substantially uniform and homogeneous, and useful for its intended purpose. By an analogous method I can fill or repair holes, cracks, etc. which extend through the thickness of metal belts or sheets and unite discrete pieces whether for patching holes, joining ends of strips, or for other purposes. I have also found that, by the methods of the present invention as hereinafter more particularly described, I can repair or patch surfaces electroplated with chromium, even when worn, cut or etched through the plate into ferrous base metal, so that, assuming the surrounding portions of the original plate to be properly ad-

herent to the base metal, the patch becomes in effect a part of the original plate, and the surface becomes substantially the same as though the defect had never existed. Further, in accordance with the present invention this filling or patching operation can be accomplished with such efficiency, rapidity, and convenience as to furnish a practical means for securing and maintaining the necessary degree of perfection in extensive metallic surfaces such as those required for the aforementioned casting purposes.

Though all highly finished metallic surfaces of large extent are subject to defects such as those mentioned, surfaces plated with chromium are particularly subject to such defects, due to the well-known and characteristic difficulties encountered in chromium plating. My invention, therefore, though applicable to the filling of defects in and with various metals, has one field of particular utility in connection with the filling with chromium of defects in a chromium plated surface.

This filling of defects in a metallic surface is accomplished according to the present invention by first mechanically shaping the defect, if not already of a form suitable for the electrolytic repairing operation, so that it forms a concavity or depression in the surface, the least width of which is great in comparison to its depth. This concavity is made to present an unbroken metallic, or electrically conducting, surface for the reception of a continuous layer of the metal to be deposited. If it is undesirable to make the concavity as deep as the defect, the continuity of the electrically conducting surface may be secured by using a closely fitting metallic plug to fill the defect up to the level of the bottom of the concavity. In working on thin metal (such as the metallic belts described in Patent No. 1,719,166), small holes may be plugged as described or, when larger areas are to be filled, a metallic backing plate may sometimes be used to give the necessary continuity to the conducting surface of the concavity, or an inlay of similar thin metal can be fitted in the hole to reduce the area to be filled to a crack, which is then filled as hereinafter more fully described.

This concavity is then constituted one electrode in an electrolytic cell or, if formed in an extensive surface, is advantageously incorporated as one wall of an electrolytic cell of commensurate size. Its surface is then electrolytically prepared by appropriate methods so that the subsequently deposited metal may be firmly adherent, after which a plating current is passed through the cell to the metal surface of the concavity until the deposit has reached a thickness adequate to at least fill the depression up to the level of the required surface. In case of thin belts or sheets of metal, if the exposed plug is objectionable on the back of the sheet, a concavity can be formed around the plug on that side of the sheet also and electrolytically filled in the manner described. In case of a chromium plated surface which has been worn, peeled, cut, or etched through to a ferrous base, or in which the bottom of the concavity has been filled with an iron plug of material size, I find that in order to secure satisfactory adherence of the electrodeposited metal, the current density should be controlled with reference to time, as hereinafter fully set forth. In patching metallic surfaces, as described, the conditions of deposition are in general most advantageously se-

lected to give a deposit as nearly as possible like the metal being patched. In patching chromium plate, or other electrolytically formed metal surfaces, if the conditions under which the original surfaces were deposited are known, best results are secured by depositing the patch under as nearly as possible identical conditions. During the chromium plating operation, the solution of the electrolyte used not only fills the cell, which is ordinarily relatively small, but is caused to flow through the cell, advantageously at a rapid rate, washing over the surface of both anode and cathode. After the required thickness of metal has been deposited, the cell is dismantled and the excess metal is mechanically removed down to the desired surface level.

The process and apparatus used will be more fully described by reference to the accompanying drawings, in which:

Fig. 1 is a schematic and greatly enlarged cross section through a defect in a plated metal surface.

Fig. 2 is a similar cross section through a defect showing where additional metal is deposited when attempting to fill or cover such defect by the customary plating procedure.

Fig. 3 is a section of a similar defect after mechanical shaping in preparation for local plating, showing the anode in position.

Fig. 4 is a similar section of a defect prepared for the plating operation, in which the lower part of the defect has been filled in order to reduce the amount of electrodeposition required.

Fig. 5 is a section of the defect shown in Fig. 4, after filling by electrolytic deposition.

Fig. 6 is a section of the same defect after the excess metal has been removed and the entire patching operation has been completed.

Fig. 7 is a cross section, on a much smaller scale, of a type of electrolytic cell used in the filling of small defects, shown in place over a defect in a flat surface.

Figs. 8 and 9 are two views of a modified form of cell used for filling elongated cavities such as cracks or scratches.

Fig. 10 is a typical wiring diagram for the apparatus used.

Fig. 11 is a diagram showing the current densities used plotted against time, for a typical defect filling operation on chromium plate.

Figure 12 is a diagrammatic representation of one form of fluid circulating system for maintaining a flow of electrolytic solution through the plating cell.

Fig. 13 is a fragmentary cross section of a metal sheet or belt at an opening which extends therethrough.

Fig. 14 is a section of the same after a depression has been cut extending in opposite directions from the opening and the opening itself has been filled with electrically conducting material flush with the bottom of the depression.

Fig. 15 is a section of the same after the electrolytic filling of the depression.

Fig. 16 is a section of the same after the sheet has been turned over and a depression has been cut on the opposite side.

Fig. 17 is a section of the same after electrolytically filling the second depression.

Fig. 18 is a section of the same after dressing down the deposits to level of the adjacent surfaces of the sheet.

Fig. 19 is a section similar to Fig. 14 but showing the opening filled flush with the surface of the sheet with no depression.

Fig. 20 is a cross section of the parts shown in

the preceding figure after the electrodeposition of metal across the opening.

Fig. 21 is a section of the same after the sheet has been turned over and a depression has been cut in the opposite side.

Fig. 22 is a section of the same after this depression has been electrolytically filled with metal.

Fig. 23 is a fragmentary sectional view of abutted edges of two sheet metal parts mounted in preparation for the electrolytic closing of the opening between them.

Fig. 24 is a fragmentary sectional view showing an inlay fitted into a hole in a metal sheet the parts being mounted in coplanar relationship on a more rigid block.

Fig. 25 shows the same parts after being joined by electrodeposited metal, mounted on a backing plate in preparation for cutting a depression in the opposite side and electrolytically filling it with metal.

Because of its especial utility in connection with the filling of defects in chromium plate, the invention will now be described as embodied in a process and apparatus particularly adapted to this use.

Referring to Figs. 1 to 6 of the drawings, the basis metal 21 is shown covered by a layer 22 of chromium in which there is a defect 23 in the form of a pit or crevice which may be supposed to have had its origin in a microscopic defect, pit, scratch, or bit of slag, etc. 24 in the basis metal 21. Any attempt to fill or cover this defect by further deposition of chromium in the usual manner, results in the preferential deposit of metal 25 at the edges 26 of the defect, which simply serves to accentuate rather than cure the defect.

In order to make possible the deposition of metal to fill the defect solidly to the bottom, I first grind or polish out the defect until solid metal is reached, cutting into the basis or backing metal if necessary and giving the defect the form of a concavity 30 (Fig. 3) whose width is materially greater than its depth. In order to further hinder the preferential deposit of metal at the edges of the depression, these edges may be given a gently rounded contour as shown at 31 in the figure. Above this is located the anode 33 which is advantageously rounded to a radius of curvature materially smaller than that of the depression 30 and is located approximately centrally thereover and closer thereto than the difference between the respective radii, so that the anode 33 is closer to the bottom of the concavity 30 than to its edges 31. Although this spacing is desirable it may be departed from to some extent, particularly when electrodepositing some metals with a better throwing power than chromium. However, it is not recommended that the distance from the anode to the center of the concavity ever be relatively very much greater than the distance from the anode to the edges of the concavity. By the means described I find it possible to so control the rate of deposit that, even with chromium, the center of the concavity is filled without undue building up of the deposit around the edges. This is believed to result from a higher density of the plating current at the center, due to the shorter distance from the anode, and to the absence of current concentration around the edges, due to their greater distance from the anode and to the rounded contour given to them.

When the defect is deep, the operation of cutting out the defect as illustrated in Fig. 3 may

require a large amount of cutting and an excessively long plating time for filling. In such cases, in order to secure a continuous electrically conducting base for the deposition of a continuous layer of electrolytic metal, it is frequently advantageous to fill in the bottom of the defect and hollow out only the part near the surface as shown in Fig. 4 rather than to cut down to solid metal as in Fig. 3. This not only eliminates most of the cutting but very greatly reduces the plating time required to fill the cavity. The filling material 35 may be lead, but if lead is used great care must be exercised to prevent the sides of the concavity from being smeared with lead, since such smears serve to prevent adherence of the deposited metal. Copper fillings I find are not ordinarily satisfactory for use with chromium plate as the copper, unless protected, becomes damaged by the electrolytic preparation process hereinafter described. Nickel and iron fillings have been found satisfactory though care must be taken to prevent a tightly driven plug from cracking the chrome plate surrounding the hole and causing it to spall off. When iron plugs are used it may be found convenient to drill out the defect to fit the plug, as indicated in Fig. 4. Otherwise the plug may be fitted into the defect as indicated in Figs. 5 and 6. The plug used should be carefully and securely driven into place so that no openings are left between it and the surrounding metal. The proportion of the depth which may be filled mechanically and that which must be cut down depends on the width of the defect and the type of filling used. With fillings having little mechanical strength, such as lead, the depth of the depression 30 is advantageously as much as three times the width of the top of filling 35. On the other hand, with stronger fillings, such as iron, the depth of the depression 30 may sometimes safely be as little as the width of the top of filling 35. The interior of the concavity should then be smoothed and cleaned, and the edges 31 rounded off as and for the purpose described.

This smoothing and cleaning of the interior of the concavity should be carried out with great care in order to provide the concavity with a smooth, continuous, uninterrupted electrically conducting surface throughout its entire area. Any abrupt change in slope or in surface level at any point in the concavity or at its edges should be completely polished out. Any surface discontinuities such as minute (or larger) cracks or crevices, or even slight differences in surface level, between the filling in the bottom of the concavity and the adjacent metal, or at any other part of the concavity, should be carefully eliminated. Any dirt, grease, metallic oxides, or other deposits which might interfere with the uniform electrical conductivity of the surface of the depression should be completely removed therefrom.

With the anode 33 located as described and as illustrated in Figs. 3 and 4, both the anode 33 and the concavity 30 are submerged in a usual type of chromium plating bath which is advantageously allowed to contact the original chromium surface for only a relatively short distance beyond the edges 31 of the concavity 30. I find that the successful filling of the concavity is much more certain, the deposited metal more sound, and the time required to fill the concavity is greatly reduced if the bath is kept in rapid motion past both anode and cathode (concavity 30) while the plating is in progress. This may

be advantageously accomplished by taking the solution from a supply reservoir and passing a rapidly flowing stream over and between the electrodes and thence returning the solution to the reservoir for reuse. The fluid velocity through the plating cell should be high enough to give turbulent flow through the cell. Higher velocities have ordinarily been found to make possible higher current densities and higher rates of deposit and thus shorten the time required for filling a given size of cavity with a given metal. Suitable velocities depend on the metal being deposited, the type and temperature of the solution used, the current densities and plating rates, etc. For filling concavities of the order of  $\frac{1}{8}$  inch in width in chromium with electrolytically deposited chromium, I find a fluid velocity of the order of 15 feet per second to be satisfactory, though with other metals, such as nickel, materially lower velocities may be used. These high velocities make possible the use of current densities much higher and rates of chromium deposit much more rapid than are otherwise attainable.

The temperature of the bath and electrodes may be chosen from a wide range as is well known in the art. Because of the known fact that higher current densities and consequent higher rates of deposition are possible at higher temperatures, the use of such temperatures is often advantageous. When, on the other hand, as is often advantageous for reasons hereinafter explained, subatmospheric pressure is maintained in the plating cell, temperatures high enough to cause boiling or cavitation in the cell or other parts of the circulating system should be avoided. The temperature once selected should be maintained within rather close limits during the plating operation, as is well understood in the art.

Even though the concavity to be filled has been thoroughly cleaned mechanically and by washing with solvents to remove grease, etc., I find that an electrolytic "preparation" operation is ordinarily advisable to insure a satisfactorily adherent deposit. For this purpose I prefer in the case of chromium to start the operation with a reverse current, temporarily making the surface to be plated the anode. As is well understood, care should be taken to avoid excessive strength or duration of this reverse current to avoid unnecessary eating away of the metal.

After this anodic preparation, the surface to be plated is made cathode by reversing the direction of the current. Under the conditions described, this change is advantageously made quickly since I have frequently observed poor adhesion of the deposit in cases where much more than one second was allowed to elapse during this reversal of the current.

I have now made the further discovery that a high quality adherent deposit of chromium can be secured, even when the steel base metal is exposed through, or adjacent to, the original chromium plate. This can be accomplished, I find, by, immediately following the anodic preparation of the surface, with current of somewhat less than minimum plating density passed through the chromium plating solution to the surface of the depression as cathode for at least a short time before increasing the current density to a value at which deposition of chromium takes place. As is well known in the chromium plating art, no matter what the applied voltage, no metal will be deposited on any part of the cathode where the current density is below a minimum value which is dependent on the temperature, 75

composition, and proportions of the bath, etc., but is fixed for each specific set of conditions and can be readily determined by routine tests. If at any point on the cathode surface the current density is not above this value, no metal whatever will be deposited at that point. The term "minimum plating density" as used in the present specification and claims to define the current density on the cathode, means the current density below which no chromium is deposited on the surface of the cathode, from the plating bath employed at the temperature used and under the other conditions obtaining.

With any given chromium plating solution, temperature, and other operating conditions the required duration of the less-than-plating-density current can be readily determined by trial. In some cases only a few seconds may be required whereas in other cases 30 to 60 minutes or more may be desirable, as no harm appears to result if the time is extended beyond the minimum requirement.

After the current of less than minimum plating density has been passed for the required time, as described, the current density is increased to the working value. As hereinbefore stated, uniformity of the patched surface is most conveniently secured by substantially duplicating the current density and other conditions used in depositing the original plate. With this limitation the working value of the current density is advantageously as near as possible to the maximum at which an unburned deposit is secured, as the plating time is thereby reduced. When the desired depth of deposit is secured, the plating is discontinued and the plating bath, the anode and all connections are removed as hereinafter more particularly described, leaving the patch as illustrated in Fig. 5. The surface is then cleaned and the excess of deposited metal mechanically cut down to the level of the surrounding surface and finished as desired, leaving a smooth continuous surface at the original surface level, as illustrated in Fig. 6.

The described changes in current direction and density, with time, are graphically illustrated in Fig. 11 which shows the values of current direction and density, plotted against time, in a typical defect-filling operation on chromium plate at a temperature of 160° F.

Referring to Fig. 11 it will be seen that a current of approximately the minimum plating density is allowed to pass in reverse direction for about one minute, that the direction is then quickly changed and a current of density slightly below the minimum plating density is passed in the normal direction for approximately 20 minutes. The density is then increased to an effective plating value. I have found that when this increase is made gradually in the normal manner as shown by curve A, the deposit is satisfactorily adherent, but when the excess deposit is polished off, a ring of what appears to be metal of a different structure is evident around the edge of the defect. I have further found that if the increase to maximum current density is made quickly, as indicated by curve B, this ring structure is absent and the deposited metal appears to be homogeneous and integral with the original chromium. Then when the excess metal deposited has been polished off, it is found to leave a surface on which the old and new metal appear to be uniform in smoothness and structure. Alternatively, in some cases, the reverse current may be followed directly by current of plating density as indi-

cated by curve C, though I prefer to use the current densities indicated by curves A or B, as described, in order to insure more perfect adhesion.

Since the conditions under which the original plate was deposited may not be known, it may not be possible to duplicate them exactly in making the local deposit, which may therefore differ slightly from the original plate in some little understood manner. As a result, the local deposit when polished off to the level of the original metal may reflect light in a slightly different manner, thus appearing, when viewed from some angles, as a spot on the surface, but for all practical purposes the old and new metal appear to be integral and homogeneous.

The apparatus of the present invention used in carrying out the process described can be varied to suit the conditions. Fig. 7 shows in cross section one form of apparatus found well suited for use in filling small circular or nearly circular depressions in chromium plate. Referring to this figure, which is drawn to a much smaller scale than Figs. 1 to 6, the chromium plate 22 is shown as a single line on the surface of the base metal 21. The anode 33 is supported centrally over the polished-out concavity 30 by means of a cell body 40. This may be composed of a non-conducting substance such as glass or a synthetic resin which is not attacked by the chromic acid bath, or it may be composed of a non-reactive metal such as lead, if provisions are made to insulate it electrically from the surface 22 and from the anode 33. A washer 41 is used to prevent leakage between cell body 40 and surface 22. This washer may advantageously be made of a synthetic rubber-like composition which is not affected by the chromic acid, is a good dielectric, and possesses sufficient plasticity to form a good seal. I have found synthetic rubber-like compounds of the polyvinyl chloride type well suited to this purpose. The washer 41 is cut out to form part of the walls of the electrolytic cell 42. It serves to insulate the body 40 (if made of metal) from the metal cathode surface 22, to prevent inward leakage of air (when the system is maintained at subatmospheric pressure), to prevent outward leakage of fluid, and to prevent contact of the bath with the surface 22 beyond the area on which a deposit is desired. To assist in the last-named function, the surface of the metal 22 where a deposit is not wanted and that of washer 41 may be painted with a "stop off" compound of known type before the apparatus is assembled.

The anode 33 extends into the cell 42 through an opening 43 in body 40. If body 40 is made of metal or of a non-yielding substance such as glass, a positive clearance is usually necessary at this point. The anode is held in place and sealed against leakage of air or of electrolyte by a rubber packing 44, which may be protected from the chromic acid by a washer 45 which may be made of the same acid-resistant material as washer 41. The anode 33 may be made of any material customarily used for anodes in chromium plating, I find lead well suited to the purpose. It extends through the rubber packing ring 44 and may be provided with a handle 46, which may be of a more rigid metal, by which the distance of the anode 33 from the concavity 30 may be adjusted by hand. The necessary electric connection may be made to handle 46 by a suitable clamp 47 and wire 48, leading to a suitable source of current

5 49. The cell may be held in place on surface 22 by means of a pressure block 50 and screw 51 which may be held in a member 52 which may be any part that is or may be fixed with reference to the surface 22.

The electrolytic cell 42 is provided with an inlet conduit 55 and an outlet conduit 56 through which a continuous flow of the electrolytic solution may be passed into and out of the cell 42. The cell 42 itself is advantageously of small volume so that high fluid velocity may be maintained therein. The conduits 55 and 56 are advantageously pointed directly at anode 33 and cathode 30 so that the stream of liquid continuously washes the surfaces of both electrodes. The abrupt change in direction of flow illustrated in this figure is also of advantage in assuring turbulence of flow in the cell 42.

20 For filling elongated defects such as cracks and scratches a modified type of cell such as that illustrated in Figs. 8 and 9 may be used. These figures are longitudinal and transverse sectional views respectively of one form of apparatus used for this purpose. They show the apparatus clamped onto the same chromium plated surface 22 of base or backing metal 21. The concavity 130 is the result of cutting out a crack or scratch in the manner described so that its width is great in proportion to its depth and the edges advantageously have rounded form. The anode 133 is elongated in form to correspond with the concavity 130. The body 140 of the cell is of a correspondingly elongated form. Both anode 133 and cell body 140 are, in this case, advantageously made of lead which permits them to be bent to conform to the curvature of any crack or scratch which may require filling. The cell body 140 is, as before, sealed against and insulated from surface 22 by a synthetic rubber-like washer 141 which is cut out to form a part of the walls of cell 142. The opening 143 with the rubber packing 144 and synthetic rubber-like washer 145 permit T-shaped handles 146 to enter the cell and grip the electrode 133, whereby the distance between anode 133 and cathode 130 can be adjusted as and for the purpose previously described. The solution of electrolyte flows through the cell from inlet 155 to outlet 156. A clamp 47 serves as before to connect the anode to wire 48 leading to a suitable source of current 49. The cell is held in place as was cell 40 by means of a pressure block 150 and screw 151 in member 152 which may be any part suitably fixed with reference to surface 22.

55 The chromic acid plating baths used are not only highly corrosive to hands and clothing of operators but even damage the surface of the metallic chromium plate. It is therefore highly desirable to prevent leakage of the solution from the cell and other parts of the apparatus as well. 60 This is most readily and effectively accomplished by maintaining subatmospheric pressure within the cell and all parts of the circulating system subject to leakage, so that the circulation through these parts of the system is maintained by suction rather than positive pressure. It is ordinarily also advantageous to maintain the surface being plated in a vertical or an inverted position.

65 The circulating system itself does not form a part of the present invention and any suitable type may be used. One type which is adapted to the simultaneous filling of a considerable number of defects is illustrated in Fig. 12 in which a tank 60 is provided for storage of the plating bath. 70 This tank should be made of material which will

be substantially unaffected by and will not significantly affect the composition of the plating bath. I find a high silicon acid and corrosion-resistant iron suitable for the tank and for other parts in contact with a chromic acid bath of the sulphate type. This tank is provided with a vent 61 to atmosphere. The plating bath is circulated by a suitable pump 62 which delivers fluid through pipe 63 into tank 60. By suction the pump 62 draws fluid from tank 60 through conduit 64 to header 65 from which individual tubes 66 lead to each of a plurality of cells 40 and/or 140. The fluid after passing through the cells 40 passes through tubes 67 and is advantageously discharged through nozzles 68 into glass chamber 69 from which it flows through pipe 70 and valve 71 to the pump 62 which returns it to tank 60 as described. The tubes 66, 67 are advantageously made of a synthetic rubber-like compound of a type such as that already described. The glass chamber 69 is provided so that watch may be kept on the flow through each individual cell to assure satisfactory results in each. A valve 72 may be provided for draining the tank when desired. It will be apparent that the pressure in the entire system from conduit 64 through the cells 40 to the pump 62 is subatmospheric. Any leakage will therefore be inward leakage of air and not outward leakage of the chromic acid bath. Damage to the surrounding chromium plate and injury to the person or clothing of the operators is thereby avoided. In using this apparatus, when the plating is completed (as determined from a knowledge of the depth of the depressions to be filled and the current densities used and resulting rate of deposit), vent valve 73 on header 65 is opened thus breaking the vacuum in the system and allowing the individual plating cells to be sucked dry. In cases where only one cell is desired to be shut down at a time, this is done by clamping shut the inlet tube 66 leading to the cell, then slightly loosening the cell from the surface 22, allowing air to leak in. As soon as the cell and outlet tube 67 are sucked dry the outlet tube is also clamped shut. The system as a whole can then continue to function with the remaining cells still in operation. Also a coil 75 may be provided in tank 60 for controlling the temperature of the bath in a known manner.

Fig. 10 shows the electrical connections used. The cell represented by anode 33 and cathode 30 cut in the surface 22 is supplied with current from any suitable source such as battery 49, the positive pole of which is connected through adjustable resistance 81, ammeter 82 and reversing switch 83 to anode 33. The cathode 30 is connected through switch 83 to the negative pole of the battery. In starting, the switch 83 is reversed for a short time, as described, making 30 the anode and 33 the cathode, but switch 83 is soon thrown to the normal position shown in the figure. When a plurality of cells are used simultaneously, as described, a separate circuit can be provided for each, or all can be supplied from a single source of current, as will be well understood by those skilled in the art. I prefer, however, to supply each cell with its own ammeter 82, and adjustable resistance 81, so that the individual current densities can be controlled to appropriate values.

The invention as so far described is embodied in a method of filling defects in the surface of thick metal such that only one surface thereof required consideration. This is however not always the case, particularly in the case of metal

sheets or casting belts to which reference has already been made, and the invention will now be described as embodied in a method of closing small or narrow holes or openings which extend 5 through the thickness of such sheets or belts.

Fig. 13 shows a cross section through a metal sheet 201 exposing an opening 202 extending through the sheet. This may be polished out to form a depression or concavity 203, and the hole filled with solder or other electrically conducting material at 204 (Fig. 14) flush with the surface of the depression as already described. If the surface of the sheet and the repair metal to be used 10 are not of chromium the rounding of the corners 205 is less necessary than in the case of chromium and may sometimes be omitted.

The filling of the depression 203 may be carried out as hereinbefore described, if the surface and the repair metal are chromium. If of other metal, 15 such for example as nickel, the preparation cycle to render the deposit adherent and the methods of deposition, will be adapted to the particular metal being used in accordance with known principles. The high velocity of the electrolyte 20 through the cell is usually unnecessary in such cases and if the cell is of considerable size, even the circulation may not be required. After deposition the part appears as shown in Fig. 15. If the exposed filling 204 is objectionable on the 25 reverse side of the sheet, the sheet is turned over and the filling 204 is preferably, though not always necessarily completely cut out to form a new depression 207 substantially opposite to the filled depression as shown in Fig. 16. The smooth uninterrupted electrically conducting surface of depression 207 is formed partly of the metal of the sheet 201 and partly of the electrolytically deposited metal 206. This is prepared for the reception of an adherent deposit and electrolytically 30 filled with repair metal 208 in the manner already described. It then appears as illustrated in Fig. 17. If smooth surfaces are desired on each side, the projecting parts of the deposits 206 and 208 may be mechanically dressed down to the planes 35 of the adjacent surfaces, though the dressing down of the first deposit 206 may frequently be more desirably accomplished prior to the cutting of the depression 207 on the opposite side.

Although the depressions 203 and 207 on opposite sides of the sheet have been shown in the drawing as of approximately equal depth this is not necessary as the depths may differ if desired. For example, if one of the surfaces carries an electroplate of chromium or other metal the depth 55 of the depression on that side is advantageously about equal to the thickness of the electroplate and is filled with an electrodeposit of metal which is the same as the electroplate, while the depression on the other side is advantageously filled with metal which is the same as that forming the body of the sheet. In the case of sheets composed of a single metal throughout their thickness, the first side operated upon need have no more depression than is inevitably formed by the mechanical and/or electrolytic preparation for reception of an adherent electrodeposit. This extreme difference between the depressions on the two sides is illustrated in Figs. 19 to 22, inclusive. In this case the opening in sheet metal 211 is filled with electrically conducting material at 214 flush with the upper surface of the sheet. A limited area of the surface surrounding the filling material 214 is blocked off by stop off varnish 215 or the like as shown in Fig. 19, and is prepared for the reception of the required elec-

trodeposit. Metal 216 is electrodeposited over this limited area as shown in Fig. 20. The sheet is then turned over and the filling material and adjacent metal of the sheet is mechanically cut out to form a depression 217 which cuts completely through the sheet into the electrodeposit 216, completely removing the filling material 214 (see Fig. 21). This depression then has a smooth, continuous, uninterrupted electrically conducting surface and is electrolytically filled with metal 218 as in the previously described embodiment and illustrated in Fig. 22. The surplus metal can then be mechanically removed, if desired, to the level of the adjacent surfaces as indicated by the broken lines in the figure.

It can be seen from Figs. 13 to 22 that the process of closing openings in sheet metal can be used without essential change regardless of whether the opening is a round hole or an elongated crack or slot or the opening between abutted edges of discrete sheets or parts. If the process is used to electrolytically join the sides of long tears or slits or the edges of discrete sheets, it is desirable to solder or cement the metal adjacent the abutted edges 221, 222 to a more rigid block or bar 223 as illustrated in Fig. 23. The process is then carried out as described with reference to Figs. 13 to 18 or Figs. 19 to 22, as desired.

This method of uniting discrete parts may be used to unite the ends of strips to form endless belts but it has a particular utility in patching large holes in metal belts or sheets, as shown in Fig. 24. The sheet 231 has a large hole into which a patch or inlay 232 of the same material and thickness is fitted. Both are soldered or cemented to a suitably rigid block or bar 233, to hold them firmly in the same plane while the opening between them is being filled with solder or other electrically conducting material 234, and until they are rigidly united by the first electrodeposit 235 as in Fig. 15 or Fig. 20. If the sheet 231 is not then sufficiently rigid to permit satisfactory handling in the further steps of the process the other side may be mounted on a relatively rigid block or bar 236 with suitable spacers 237 interposed as shown in Fig. 25. While so mounted the depression on the second side is cut out and electrolytically filled, and if desired, dressed down to the level of the surface of the sheet as already described.

The application of the process will be better understood from the following examples, the first six of which illustrate its use in the successful filling of cavities in chromium plate while the last two illustrate its use in patching of thin sheets or belts of nickel:

#### Example 1

- Composition of plating bath—Chromic acid 250 g. per liter; boric acid 30 g. per liter; sulphate ions= $\frac{1}{100}$  of hexavalent chromium ions.
- Temperature of bath 160° F.
- Diameter of concavity to be filled 0.062 inch.
- Depth of concavity 0.0015 inch.
- Filling in base of defect—iron.
- Distance between electrodes  $\frac{1}{8}$  inch.
- Current densities—Reverse 38.2 amperes per square foot for 1 minute, quickly changed to direct 39.8 amperes per square foot for approximately  $\frac{1}{2}$  hour, then gradually increased over about 40 minutes to direct 540 amperes per square foot for  $1\frac{3}{4}$  hours.
- Total time  $2\frac{1}{4}$  hours.

- Results—good adherent plate. Ring visible just inside edge of filled cavity after excess metal dressed off, but no other indication of lack of homogeneity.

#### Example 2

- Same as Example 1 except that increase from 39.8 amperes per square foot to 540 amperes per square foot was made quickly (as rapidly as rheostat could be set) instead of over a period of 40 minutes. Results the same except that no ring structure was visible.

#### Example 3

- Composition of plating bath same as in Example 1 except that sulphate ions= $\frac{1}{50}$  of hexavalent chromium ions.
- Temperature of plating bath 160° F.
- Diameter of concavity to be filled 0.15 inch.
- Depth of concavity to be filled 0.007 inch.
- Filling in base of defect—lead.
- Distance between electrodes  $\frac{1}{8}$  inch.
- Current densities—reverse 19.7 amperes per square foot for 1 minute, quickly changed to direct 19 amperes per square foot for  $\frac{1}{2}$  hour, increased over a period of about 40 minutes to direct 400 amperes per square foot for  $7\frac{1}{4}$  hours.
- Total time  $7\frac{3}{4}$  hours.
- Results—good adherent plate. Ring visible as in Example 1, but no other evidence of lack of homogeneity.

#### Example 4

- Composition of plating bath same as in Example 3.
- Temperature of plating bath 160° F.
- Concavity (scratch) width  $\frac{1}{16}$  inch, length  $1\frac{1}{2}$  inch.
- Depth of concavity 0.0005 to 0.0015 inch.
- Filling not needed.
- Distance between electrodes  $\frac{1}{8}$  inch.
- Current densities same as Example 1 except plating current on for  $2\frac{1}{2}$  hours.
- Total time 3 hours.
- Results good adherent plate. Ring visible but apparently of no practical significance.

#### Example 5

- Composition of plating bath same as in Example 3.
- Temperature of plating bath 164° F.
- Concavity—diameter  $\frac{1}{16}$  inch.
- Concavity—depth 0.003 inch.
- Filling not needed.
- Distance between electrodes  $\frac{1}{8}$  inch.
- Current densities same as Example 1 except plating current 523 amperes per square foot for  $4\frac{1}{2}$  hours.
- Total time 5 hours.
- Results same as Example 1.

#### Example 6

- Composition of plating bath—Chromic acid 250 g. per liter; sulphate ions= $\frac{1}{55}$  of hexavalent chromium ions.
- Temperature of bath 170° F.; of plate 185° F.
- Diameter of concavity  $\frac{1}{16}$  inch.
- Depth of concavity 0.006 inch.
- Filling in base of defect—iron.
- Distance between electrodes  $\frac{1}{4}$  inch.
- Current densities—reverse current 100 amperes per square foot for 2 minutes, quickly changed to forward current 30 amperes per square foot for 1 minute, quickly increased to forward current 2000 amperes per square foot for 57 mins.

8. Total time 1 hour.  
 9. The deposit was tightly adherent, bright, and matched the original plate in hardness, appearance and other properties as far as could be detected.

*Example 7*

This example involved the patching of a pin-hole extending through a hard electroformed sheet of nickel approximately 0.010 inch in thickness. The hole was filled with solder and, with a small hand grinder, a saucer shaper depression was hollowed out around the filled hole as shown in Fig. 14, the solder filling being flush with the bottom of the depression. In the filling operation care was taken to avoid flux pockets particularly between the solder filling and the sides of the hole and to limit the area and degree of heating to prevent distortion of the sheet. The surface of the nickel in the depression surrounding the solder filling was first scraped as free as possible of excess solder and was further polished using sandpaper of increasing fineness. The polishing of the nickel surface of the depression was completed by use of a paste of diatomaceous earth and water and clean cloth. The surface was then electrolytically prepared for reception of an adherent electrodeposit, by anodic treatment in a strong solution of sulfuric and phosphoric acids. Because of the large extent of the surface of the sheet this treatment and the subsequent electrodeposition were carried out in a small cell set up and clamped in place, with an interposed rubber gasket or the like, on the sheet metal surface and including the depression and immediately surrounding surface. After the anodic treatment the cell and surface were thoroughly rinsed with water. The plating current was then started simultaneously with the introduction of the nickel plating solution into the cell, care being taken in the process to avoid excessively high current density on any part of the surface. After the lowest part of the deposit had reached the level of the adjacent surface of the sheet as shown in Fig. 15 the operation was stopped, the solution removed from the cell and the cell removed from the sheet. The protruding parts of the deposit were dressed down to the level of the surrounding surface and the sheet turned over. The hand grinder was then used to form a depression opposite the filled depression, removing all of the solder filling 204 (Figs. 15 and 16). The newly formed depression had a continuous smooth nickel surface throughout its extent, composed partly of the nickel of the sheet and partly of the nickel electrodeposit. This depression was then polished, prepared, and filled with nickel in the same manner as was that on the first side. The surplus electrodeposited metal was then mechanically dressed down, giving the patch the same thickness as the sheet itself. The patched sheet was then substantially uniform and homogeneous, and when given the desired surface finish, was suitable for use as a casting surface for films or coating on paper.

*Example 8*

This example involved the repair of a damaged and punctured portion of a large electroformed sheet of hard nickel approximately 0.015 inch in thickness. The puncture appeared to have been made by a blunt object which stretched and distorted the metal surrounding the puncture itself, so that the metal could not be crowded back into the plane of the original sheet. The first step in the repair involved the removal of the entire

70 75 77 79 80 81 82 83 84 85 86 87 88 89 90 91 92 93 94 95 96 97 98 99

distorted area by a circle cutter, in a manner to cause no further distortion. This resulted in a circular hole approximately two inches in diameter in a flat nickel sheet. A two inch circle of nickel was cut from a sheet of the same character and thickness and fitted into this hole. Both pieces were then cemented in a coplanar position on a heavy block of steel as illustrated in Fig. 24. In order to prevent further distortion of the metal this cementing operation was accomplished with a commercial thermoplastic cement softening at about 100° C. The crack between the patch and the sheet was filled with solder as at 234 taking care to avoid flux inclusions and overheating of the metal. The central part of the patch and the surface of the sheet surrounding the hole were painted with stop off varnish, as at 215 Fig. 24, leaving an exposed annular surface of metal extending for a short distance on each side of the solder ring. This annular area was polished and electrolytically prepared and a layer 235 of nickel of about 0.020 inch thickness was deposited thereon, in the manner described in the previous example. The solution and cell were removed and the now united parts were removed from the backing plate by softening the thermoplastic cement. The sheet was then turned over and cemented to the flat surface of a backing plate 236, as indicated in Fig. 25, with interposed spacers 237 to provide room for the electrodeposited ring 235, which was smoothed down on the level of the surface of the spacers before cementing to the backing plate. Thereafter the solder was mechanically cut out to form an annular depression as indicated in Fig. 21. The surfaces were painted with stop off varnish as before, the annular surface of the depression was polished and prepared, and nickel was electrodeposited therein from a solution and under conditions as nearly as possible duplicating those used in the electroformation of the sheet. Before removal of the sheet from the backing plate and while the sheet was still held firmly in a plane position the electrodeposited ring was dressed down to the level of the surrounding surface. The backing plate was then removed by heating to about 100° C. to soften the cement used, and the newly finished surface was cemented to the plane surface of a similar backing plate to hold the belt firmly while the initial annular deposit 235 was dressed down to the level of the surface of the sheet. The patched sheet was then of substantially uniform thickness and substantially homogeneous throughout, the surface was uniformly smooth, and no evidence of the patch was apparent. Tests indicated that every part of the patch met the specifications for strength and hardness established for the sheet itself.

In the case of a chromium plated surface where there has been local peeling off of the plate, a satisfactory repair may be made if the surrounding portions of the plate are adequately adherent to the base metal, by polishing out the peeled area, rounding off the edges of the surrounding plate, and then completing the repair as described.

In the case of worn chromium plated gages and other tools, the natural wear is frequently found to have given the worn area the form of a wide shallow depression such as is required for the patching operation herein described, and has, in general, the form illustrated to a greatly distorted scale by the solid lines in Fig. 3. In such cases, the operation of forming the concavity may be omitted, having been in effect accomplished by

the wear which necessitated the repairs. The area may then be cleaned and the repair may be made in the manner described. The process of the present invention then results in an adherent patch even though the plate may have been worn through to the steel base or been cut or etched through to it in the process of preparing the area for plating, in distinction from prior practice which, under such conditions, required the stripping off of all chromium and completely new plating.

The process as described also serves to produce an adherent chromium plate in cases where the original chromium plate has been worn or cut through into a nickel instead of an iron base, or where it has been cut through a nickel underlayer into a ferrous base. Also, as hereinbefore stated, nickel plugs may be used to fill the bottom of the cavity where desired.

In cases where the parts are relatively small and the concavities to be filled are shallow, local plating cells such as illustrated in Figs. 7, 8, and 9 may not be necessary, and the repair may be made, if desired, by plating over both worn and unworn parts by the use of conventional plating equipment, using a stop-off in the known manner where no deposit is desired.

Further, use of the less-than-plating-density current as a preliminary to electrodeposition of chromium to fill cavities in chromium plated surfaces wherein steel base metal is exposed, can profitably be extended to the deposition of chromium on any surface of greater or lesser extent which is composed partly of chromium and partly of ferrous metal, and may on occasion be used with advantage in the initial deposition of chromium onto steel surfaces and in the deposition of additional chromium onto chromium surfaces.

The invention has been described in detail as applied to chromium plated and nickel surfaces because of what is believed to be the importance of these applications. With the principles of the invention, as hereinbefore described, in mind, those skilled in the electroplating art will readily understand how to modify the process described to adapt it to the filling of depressions in chromium and other metals with electrolytically deposited metals other than chromium or nickel as well as with these metals. For example, when depositing metals other than chromium for which the plating solutions do not have the corrosive properties found in chromic acid, subatmospheric pressure and closed electrolytic cells are unnecessary. Open topped cells may be used, with the surface to be plated frequently forming a part or all of the bottom or one side of the cell. Also in the case of metals other than chromium or nickel, the electrolytic preparation of the metal for receiving an adherent deposit will differ from those described and will be appropriate to the metal used as is well known in the art, and in plating, a simple circulation of the plating solution through the cell, or, in larger cells, agitation of the solution in the cell, may serve in place of the relatively high velocities used in depositing chromium, whereas in other cases even agitation may be unnecessary.

The term "metal" as used in the present specification and claims to define the surfaces on which deposition is to be made, or the deposit to be made thereon, is to be understood to mean a metal which by known methods can be used as a base for electrodeposition, or can be electrodeposited, respectively, and to specifically exclude metals which are such only in the chemical sense of the word.

The invention has further been specifically described with reference to the filling of small cavities in metallic surfaces and of larger holes in thin sheets. It will be appreciated that the same principles apply to the filling of depressions, cavities, or defects of almost any reasonable size and shape, and that those skilled in the art will be able in the light of the foregoing explanation, to make any changes required in the size and form of the apparatus described, in order to adapt it to the filling of a great variety of depressions and cavities in metallic or other electrically conducting surfaces. It will also be readily understood that in the electrolytic method described for closing the opening between a sheet and an inlaid patch so that the two form a single homogeneous sheet, the shape of the parts and of the line along which they are joined is immaterial to the process which can accordingly be used to join ends of strips to form homogeneous endless metal belts and to join the edges of sheets as well as to make patches of almost any reasonable shape and size. This application is a continuation-in-part of my prior co-pending application Serial No. 571,264, filed January 4, 1945, and now abandoned in favor of the present application.

I claim:

1. Electrolytic method of closing openings in metallic surfaces, which comprises: mechanically imparting to an opening the form of a depression whose depth is slight relative to its least width; filling any part of the opening which is deeper than said depression, with electrically conducting material; providing said depression with a continuous uninterrupted electrically conducting surface throughout its entire area; enclosing the electrically conducting surface of said depression in an electrolytic cell; electrolytically preparing the surface of said depression for receiving an adherent electroplate; thereafter electrolytically depositing metal in said depression, and maintaining during said electrodeposition a substantially continuous flow of the electroplating solution through said cell, submerging and washing over the surface of said depression.
2. The method of claim 1 wherein the path of the electroplating current through the electroplating solution to the lowest part of the depression is maintained definitely shorter than the path to the edges of the depression.
3. Process of electrolytically filling with metallic chromium, a defect in an extensive chromium surface, which comprises: mechanically imparting to a defective portion of said surface, the form of a depression having a width which is great compared to its depth, well-rounded edges, and a continuous electrically conducting surface throughout its extent; blocking out a restricted area of said extensive surface including and immediately surrounding said depression; fixing an electrode, of a form corresponding to that of said depression, in position over the deepest part thereof; passing a stream of chromium plating solution through the space between said depression and said electrode in a manner to submerge and wash over said electrode and the surface of said depression; electrolytically preparing the surface of said depression for the reception of an electrodeposit of chromium; and passing an electric current through said stream of electroplating solution to the surface of said depression while maintaining the length of the current path to the bottom of said depression less than that to the edges thereof.
4. Process of electrolytically filling with metal-

lic chromium, a defect in a chromium plated surface, which comprises: mechanically cutting out the defect to form a depression whose least width is great compared to its depth; filling any part of the defect which is deeper than said depression, with electrically conducting material; providing said depression with a continuous uninterrupted electrically conducting surface throughout its entire area; constituting said area one wall of an electrolytic cell; electrolytically preparing the surface of said depression for receiving an adherent electroplate; thereafter passing an electric current through said cell to the electrically conducting surface of said depression, as cathode; and maintaining, during the passage of said current, a substantially continuous flow of chromium plating solution through said cell, submerging and washing over the surface of said depression.

5. Process of electrolytically filling, with metallic chromium, a defect in a chromium plated surface, which comprises: mechanically cutting out the defect to form a depression whose least width is great compared to its depth; filling any part of the defect which is deeper than said depression, with electrically conducting material; giving the edges of said depression a well rounded form; providing said depression with a continuous uninterrupted electrically conducting surface throughout its entire area; constituting said area one wall of an electrolytic cell; passing a rapidly flowing stream of a chromium plating solution through, and completely filling, said cell, in a manner to submerge and wash over the surface of said depression; maintaining subatmospheric pressure in said cell; passing an electric current from said surface as anode, through said cell for a short time; immediately thereafter passing an electric current of slightly less than the minimum plating density to said surface as cathode, for at least a short time; then increasing the current density to that required to yield a satisfactory deposit of chromium.

6. Electrolytic method of filling defects in metallic surfaces, which comprises: mechanically forming in a metallic surface at the location of a defect, a depression having a width which is great relative to its depth; imparting to said depression a smooth, continuous uninterrupted electrically conducting surface throughout its entire area; blocking out a restricted area of said surface including and immediately surrounding said depression; constituting the electrically conducting surface of said restricted area one electrode in an electrolytic cell; providing in said cell another electrode having a form corresponding to that of said depression; fixing said other electrode in place adjacent to and over the deepest part of said depression in such position that the edges of said depression will nowhere be relatively much nearer to said other electrode than is the deepest part of said depression; electrolytically preparing the metallic surface in said restricted area for receiving an adherent electroplate; thereafter electrolytically depositing metal in said depression; and maintaining during said electrodeposition a substantially continuous flow of electroplating solution through said cell, submerging and washing over the surface of said depression.

7. Electrolytic method of closing openings in metallic surfaces, which comprises: closing the bottom of such an opening; imparting to the closed opening the form of a depression having a width which is great relative to its depth, and a continuous uninterrupted electrically con-

ducting surface throughout its entire area; blocking out a restricted area of the surface including and immediately surrounding said depression; constituting the electrically conducting surface of said restricted area one electrode in an electrolytic cell; electrolytically preparing the metallic surface in said restricted area for receiving an adherent electroplate; thereafter electrolytically depositing metal in said depression; and maintaining during said electrodeposition a substantially continuous flow of the electroplating solution through said cell, submerging and washing over the surface of said depression.

8. Process of electrolytically filling with metallic chromium, a defect in a chromium plated surface on a ferrous metal base, which comprises: cutting out the defect to form a depression whose least width is great in comparison to its depth; providing said depression with a smooth, continuous, uninterrupted electrically conducting surface throughout its extent; blocking out a restricted area of said chromium plated surface, including and immediately surrounding said depression; fixing an electrode of a form corresponding to said depression in position over and nearest to the deepest part thereof; passing a stream of chromium plating solution through the space between said depression and said electrode in a manner to submerge and wash over the surfaces of said electrode and said depression; passing an electric current for a short time from the surface of said depression as anode through said stream of chromium plating solution to said electrode; then reversing the direction of flow of current and maintaining a current density on the surface of said depression as cathode which is slightly less than the minimum plating density, for at least a short time; and then increasing the current density to one which causes the deposition of chromium in said depression.

9. Process of patching a hole which extends through a chromium plated surface to ferrous base metal, which comprises: polishing out a restricted area, including and immediately surrounding said hole, to form a depression having a depth which is small in comparison with its least width, and having a smooth, continuous, uninterrupted, electrically conducting surface throughout its extent; fixing an electrode in such relation to said depression that the distance from said electrode is less to the center than to the edges of said depression; maintaining chromium plating solution between and in contact with said electrode and the surface of said depression; passing an electric current, for a short time, through said solution from the surface of said depression as anode, to said electrode; substantially immediately thereafter passing an electric current, for at least a short time, through said solution from said electrode to the surface of said depression as cathode; maintaining the current density on said cathode, during said time, at a value somewhat below the minimum plating density; then increasing the current to a density sufficient to accomplish the deposition of chromium.

10. Electrolytic method of closing openings in metallic surfaces, which comprises: mechanically imparting to an opening the form of a depression, materially greater in width than in depth; filling any part of the opening which is deeper than said depression with electrically conducting material; providing said depression with a continuous uninterrupted electrically conducting surface throughout its area; constituting said surface of the depression one electrode in an

21

electrolytic cell; preparing said surface of the depression for receiving an adherent electrodeposit; and thereafter electrolytically depositing metal in said depression.

11. Method of closing openings which extend through the thickness of sheet metal, which comprises: forming a depression with sides sloping from said opening to the level of the adjacent surface; filling the opening in the bottom of said depression with electrically conducting material; imparting to said depression a continuous uninterrupted electrically conducting surface throughout its extent; electrolytically filling said depression with metal; forming a depression on the other side of said sheet metal opposite to said electrolytically filled depression; imparting to said second depression a continuous electrically conducting surface throughout its extent; and electrolytically filling said second depression with metal.

12. Method of closing openings which extend through the thickness of sheet metal, to render said sheet substantially homogeneous throughout its thickness, which comprises: forming a depression with sides sloping from said opening to the level of the adjacent surface; filling the opening in the bottom of said depression with electrically conducting material; imparting to said depression a continuous uninterrupted electrically conducting surface throughout its extent; preparing said surface for receiving an adherent electrodeposit; electrolytically filling said depression with metal; forming, on the other side of said sheet metal, a depression of such depth as to completely remove the filling material placed in said original opening; imparting to said second depression a continuous electrically conducting surface formed partly of the metal electro-deposited in said first depression; preparing said surface for receiving an adherent electrodeposit; and electrolytically filling said second depression with metal.

13. Electrolytic method of closing holes which extend through sheet metal, which comprises: forming a depression centered around said hole; filling the hole at the bottom of said depression, with electrically conducting material; imparting to said depression a continuous uninterrupted electrically conducting surface throughout its extent; blocking out a restricted area of the surface including and immediately surrounding said depression; constituting the electrically conducting surface of said restricted area one electrode in an electrolytic cell; preparing the surface of the metal in said restricted area for receiving an adherent electrodeposit; electrolytically filling said depression with metal; forming a depression surrounding said hole on the opposite side of the sheet; imparting to said second depression a continuous electrically conducting surface throughout its extent; blocking out a restricted area of the surface including and immediately surrounding said second depression; constituting the electrically conducting surface of said restricted area one electrode in an electrolytic cell; preparing the surface of the metal in said restricted area for receiving an adherent electrodeposit; and electrolytically filling said second depression with metal.

14. Method of welding together edges of sheet metal, which comprises: holding the edges to be joined in the relative positions they are to occupy after welding; forming a depression with sides sloping from said edges to the level of the adjacent surface; filling the opening between said

22

edges, at the bottom of said depression, with electrically conducting material; imparting to said depression a continuous uninterrupted electrically conducting surface throughout its extent; electrolytically filling said depression with weld metal; forming a depression on the other side of said sheet metal, opposite to said electrolytically filled depression; imparting to said second depression a continuous electrically conducting surface throughout its extent; and electrolytically filling said depression with weld metal.

15. Electrolytic method of welding together edges of sheet metal which comprises: holding the edges to be joined in the relative positions they are to occupy after welding; forming a depression with sides sloping from said edges to the level of the adjacent surface; filling the opening between said edges, at the bottom of said depression, with electrically conducting material; imparting to said depression a continuous uninterrupted electrically conducting surface throughout its extent; electrolytically preparing said surface to receive an adherent electrodeposit; electrolytically filling said depression with weld metal; forming, on the other side of said sheet metal, opposite to said electrolytically filled depression a depression of such depth as to completely remove the filling material placed in said original opening; imparting to said second depression a continuous electrically conducting surface throughout its extent; said surface being formed partly of the metal electro-deposited in said first depression; electrolytically preparing said surface to receive an adherent electrodeposit; and electrolytically filling said second depression with weld metal.

16. Electrolytic method of closing openings which extend through the thickness of sheet metal, which comprises: preparing, on one side of said sheet metal, a surface of limited area surrounding the opening to be closed; said preparation including the filling of said opening flush with the prepared surface, with electrically conducting material; to render the surface in said limited area smooth, continuous, and electrically conducting across said opening; said preparation further including a treatment to condition the metal of said sheet in said limited area for the reception of a metallic electrodeposit; electrolytically depositing a material thickness of metal on said area; mechanically removing said electrically conducting filling material together with adjacent metal of the sheet by cutting from the opposite side of said sheet metal to form a depression in the surface of said opposite side; said depression extending through the metal of the sheet into the aforesaid electrolytically deposited metal; preparing the surface of said depression for the reception of an adherent electrodeposit; and electrolytically filling said depression with metal.

17. Electrolytic method of welding together abutted edges of sheet metal parts, which comprises: temporarily holding said abutted edges in the relative positions they are to occupy after welding; preparing, on one side of said sheet metal, a surface of limited area extending in both directions from the line of abutment, said preparation including the filling of the space between the abutted edges flush with the prepared surface, with electrically conducting material, to render the surface in said limited area smooth, continuous, and electrically conducting across the line of abutment, said preparation further

including a treatment to condition the metal of said sheet metal parts in said limited area for the reception of a metallic electrodeposit; electrodepositing a material thickness of metal on said area; mechanically removing said electrically conducting filling material together with adjacent metal of the sheet by cutting a depression extending from the opposite side through the metal of said sheet into the aforesaid electrolytically deposited metal; preparing the surface of said depression for the reception of an adherent electrodeposit; and electrolytically filling said depression with metal.

18. Method of securing an adherent electrodeposit of chromium on at least a part of the surface of a metallic body, which surface is composed of at least one metal chosen from the class consisting of iron and chromium, which comprises a treatment consisting of the following steps: submerging the part of said surface on which the electrodeposit is to be made, in a chromium plating solution; anodically treating said part of said surface by passing an electric current through said solution from said surface as anode for a short time; following this by a cathodic treatment which is accomplished by passing an electric current of somewhat less than plating density through said solution for at least a few seconds before any application of plating density current, to improve the adherence thereto of the chromium subsequently deposited thereon; then, while maintaining the flow of current to said part of said surface as cathode, increasing the current density to a density at which electrodeposition of chromium occurs on the cathode, to initiate deposition thereof.

19. Method of securing an adherent electrodeposit of chromium on at least a part of the surface of a metallic body, which part of said surface is composed of at least one of the metals chosen from the class consisting of iron and chromium, which comprises subjecting the metal composing said part of said surface to a treatment consisting of the following steps: anodically treating said metal in a chromium plating solution, for a short time; thereafter, and prior to any application of plating density current thereto, cathodically treating said metal, in a chromium plating solution, for at least a few seconds, to improve the adherence thereto of the chromium subsequently deposited thereon; then, passing a plating current to said metal as cathode to form the desired deposit thereon; said cathodic treatment being carried out at a cathode current density somewhat less than the minimum value at which chromium will be deposited from said plating solution, and being continued until the plating current is applied and the deposition of chromium initiated.

20. Method of securing an adherent electrodeposit of chromium on at least a part of the

surface of a metallic body, which part of said surface is composed of at least one of the metals chosen from the class consisting of iron and chromium, which comprises subjecting the metal composing said part of said surface to a treatment consisting of the following steps: a short anodic treatment in the chromium plating solution; followed by a cathodic treatment of at least a few seconds duration, in said chromium plating solution, at a current density insufficient to deposit any chromium on the cathode; followed by a cathodic treatment at a current density sufficient to cause the desired deposition of chromium thereon; said cathodic treatment at less than plating density being initiated before any application of plating density current and continued until the plating current is applied.

21. Method of securing an adherent electrodeposit of chromium on at least a part of the surface of a metallic body, which part of said surface is composed of both iron and chromium, which comprises subjecting the metal composing said part of said surface to a treatment consisting of the following steps: anodically treating said metal in a chromium plating solution, for a short time; thereafter, and prior to any application of plating density current thereto, cathodically treating said metal, in a chromium plating solution, for at least a few seconds, to improve the adherence thereto of the chromium subsequently deposited thereon; then, passing a plating current to said metal as cathode to form the desired deposit thereon; said cathodic treatment being carried out at a cathode current density somewhat less than the minimum value at which chromium will be deposited from said plating solution, and being continued until the plating current is applied and the deposition of chromium initiated.

40 PHILIP S. BLICKENSDERFER.

#### REFERENCES CITED

The following references are of record in the file of this patent:

#### UNITED STATES PATENTS

| Number    | Name      | Date          |
|-----------|-----------|---------------|
| 1,090,456 | Darrah    | Mar. 17, 1914 |
| 1,285,875 | Woodbury  | Nov. 26, 1918 |
| 1,645,927 | Pierce    | Oct. 18, 1927 |
| 1,757,671 | Langseth  | May 6, 1930   |
| 1,809,872 | Soderberg | June 16, 1931 |
| 1,909,716 | Pinner    | May 16, 1933  |
| 1,918,605 | Jones     | July 18, 1933 |
| 2,063,760 | Schulein  | Dec. 8, 1936  |
| 2,293,810 | Domim     | Aug. 25, 1942 |

#### FOREIGN PATENTS

| Number     | Country       | Date          |
|------------|---------------|---------------|
| 60 154,282 | Great Britain | Nov. 8, 1920  |
| 156,999    | Great Britain | Apr. 23, 1920 |